

March 17, 1931.

E. GMINDER

1,796,598

PROCESS OF TREATING THE FIBERS OF TEXTILE MATERIAL

Filed Nov. 11, 1926



Invantor  
Emil Gminder  
by his attorneys  
Denn Fairbank Bright & Henshaw

## UNITED STATES PATENT OFFICE

EMIL GMINDER, OF REUTLINGEN, GERMANY

## PROCESS OF TREATING THE FIBERS OF TEXTILE MATERIAL

Application filed November 11, 1926, Serial No. 147,654, and in Germany November 30, 1925.

This invention relates to a new method for fiber-refining like that which is produced by the swelling of vegetable fiber material under the action of alkalies or acids. 5 The process is specially designed to improve the mercerization. It has become known that the mercerization effect is the better the lower the temperature of the mercerization liquid is, this being probably due to the 10 fact that at lower temperature the swelling effect can be obtained in a better and more perfect measure, the destroying influence of the mercerization liquid not having to be feared. The higher the temperature of the 15 mercerization liquid is the sooner begins the destroying influence of the swelling agent and destruction of the cellulose is effected rather than merely the swelling. It has been proposed to improve the mercerization 20 process by cooling in several baths during the mercerization. In all these tests it has been overlooked that a considerable amount of heat was developed by the effect of the wetting liquid on the fiber as well as 25 by the process of stretching so that during the cooling of the mercerization liquid the heat produced upon and in the fiber could not be neutralized at all or only to an insignificant degree. 30 The process which will be hereinafter described shows a way to do away with the heat from reaction during the impregnating treatment as well as with the heat produced at the stretching. The process consists in 35 conducting the fiber material over cooling surfaces subsequently to the impregnating with the liquid and subsequently to the squeezing out. Another possibility is to construct the stretching mechanism as a refrigerating device over which the material 40 is conducted.

The process may be carried out, for instance for the treatment of pieces of fabric, as follows: The piece of fabric is steeped in 45 lye, squeezed out and then conducted over cooling cylinders from which it passes through the stretching field of the neutralizing device. This process alone brings the great advantage that not all the lye has to 50 be cooled but only the lye contained in the

material, so that the piece of fabric can consequently be maintained at a much lower degree of temperature than is possible when, as has been the case up to the present, all the lye has to be cooled. The effect of the 55 process is even much more favorable if the cooling begins only with the stretching process or during the same so that not only the heat produced at the action of the lye upon the piece of textile material but also the 60 heat produced at the stretching of the piece of textile material saturated with lye is neutralized when it is being produced as in this case a substantial improvement of the effect of the mercerization and an economical working are obtained. 65

The working method is diagrammatically illustrated in several forms of execution, by way of example, in the accompanying drawings, in which:—

Fig. 1 illustrates the proceeding in chainless mercerizing machines.

Fig. 1a is a top plan view of the construction shown in Fig. 1.

Fig. 2 is an edge view of a chain mercerizing machine.

Fig. 3 is a top plan view of the parts shown in Fig. 2.

Fig. 4 shows a form of construction for cooling a continuous web of material on 80 both sides.

Figs. 5 and 5a show in side elevation and top plan view respectively an arrangement for the intentional production of a shrinking at the end of the process.

Figs. 6 and 6a illustrate in similar views to Figs. 5 and 5a an arrangement for the production of shrinking in the directions of the weft and of the warp.

Referring to Fig. 1 a,  $a^1$ ,  $a^2$  are the stretching cylinders,  $b$ ,  $b'$  are the cooling cylinders and  $g$  is the textile material conducted over the cylinders of the two groups.

In Figs. 2 and 3 the piece of textile material conducted between the clutching chains is designated by  $g$  and  $b$ ,  $b^1$ ,  $b^2$  are the cooling elements over or under which the piece of textile material passes.

In so-called chainless mercerizing machines, in which the stretching field consists 100

of spreading-out cylinders, the cooling is preferably effected by conducting the piece of textile material between the spreading-out cylinders over a cooling cylinder.

5 In chain mercerizing machines, in which the stretching field is formed by two clutching chains diverging in the direction of travel flat cooling elements are preferably arranged under or over or on both sides of 10 the piece of textile material.

As shown in Fig. 4 the textile material *g* passes over a number of cooling cylinders *a* and over a cooling cylinder *A* arranged at a variable distance from the cooling cylinders *a* so that the stretching of the material 15 may be varied. The textile material is cooled on both sides.

In the processes, which have been described above, the neutralizing procedure 20 has not been taken into consideration, as it is carried out in the well known manner, for instance by diluting the mercerizing bath by addition of hot water, when the mercerized material is still in the stretching field. 25 The mercerizing effect is made permanent by this treatment and shrinking is prevented.

A much more effective preventing of shrinking can, however, be obtained and carried through in the same way as the cooling 30 of the textile material if, instead of the treatment with hot water, dry heat is applied.

With this object in view the textile material is conducted over heat radiating elements, in a similar manner as over the cooling elements, for instance over hollow cylinders which are internally heated by steam 35 or heated liquids.

According to the invention the textile 40 material is submitted during the stretching to dry heating whereby the shrinking of the mercerized material is prevented as this shrinking occurs only at low temperature.

The degree of shrinking can be regulated 45 at will by stronger or less strong heating. If the shrinking has to be completely suppressed, diluting of the mercerizing liquid by hot liquid may be employed, besides the heating by hot cylinders.

50 This process makes it further possible to make the mercerizing effect produced on the first cooling elements permanent for a certain part and to combine the same with a shrinking adapted to be regulated in the

55 manner indicated in order to make the mercerized material more dense. In this case it is advisable to arrange cooling cylinders also following the heating cylinders in the stretching field. Following these smooth 60 cooling cylinders, there are no stretching cylinders. By the smooth cooling cylinders a shrinking in the direction of the weft and, eventually by a reduced delivering velocity, also a more or less great shrinking in the 65 direction of the warp is obtained.

Several diagrammatical illustrations in Figs. 5, 5a and 6, 6a serve to explain the character of this working procedure.

The textile material *g* is alternately conducted over stretching cylinders *a*, *a*<sup>1</sup>, *a*<sup>2</sup> 70 and cooling cylinders *b*, *b*<sup>1</sup> and then, in order to neutralize with dry heat, i. e., to counteract the shrinking process, the material is conducted over an internally heated hollow cylinder *e*, behind which a stretching 75 cylinder *a*<sup>3</sup> and a cooling cylinder *b*<sup>2</sup> are arranged, the material being then conducted over a smooth cylinder *i* which rotates at slower speed whereby the tension is reduced at the end of the proceeding and a 80 compressing or shrinking is intentionally permitted.

In a similar manner alternate in Fig. 6 first stretching cylinders *a*, *a*<sup>1</sup>, *a*<sup>2</sup>, *a*<sup>3</sup>, *a*<sup>4</sup> with the cooling cylinders *b*, *b*<sup>1</sup> heating cylinders 85 *e*, *e*<sup>1</sup> being then arranged instead of the cooling cylinders. The textile material *g* passing over these cylinders is mercerized, heated with dry heat, hot liquid being finally 90 sprinkled onto the same through nozzles *f*.

I claim:—

1. A process for the treatment of woven textile material which includes subjecting the goods to the action of a shrinking liquid, and thereafter subjecting the material to a series of alternate cooling and transverse stretching actions.

2. A process for the treatment of woven textile fabric which includes impregnating the fabric with a mercerizing liquid, squeezing out the excess liquid, and thereafter subjecting the fabric to a series of alternating cooling and transverse stretching actions.

3. A process for the treatment of woven 105 textile fabric which includes impregnating the fabric with a mercerizing liquid, squeezing out the excess liquid, and thereafter alternately cooling and transversely stretching the fabric a plurality of times.

4. A process for the treatment of woven textile fabric which includes impregnating the fabric with a mercerizing liquid, squeezing out the excess liquid, thereafter alternately cooling and transversely stretching 115 the fabric a plurality of times and thereafter heating the fabric.

In testimony whereof I affix my signature.  
EMIL GMINDER.